

## UNITED STATES PATENT OFFICE

2,113,906

## BLEACHING PROCESS

Edwin P. Sherman, Brooklyn, N. Y., assignor to  
 The Geo. E. Sherman Company, Inc., Brooklyn,  
 N. Y., a corporation of New York

No Drawing. Application March 11, 1937,  
 Serial No. 130,417

## 4 Claims.

(Cl. 8-2)

This invention relates to bleaching processes and more particularly to a process for bleaching vegetable and animal substances, such as cotton, rayon, cellulose acetate silk and wool, either 5 waste or raw or in yarn or piece goods.

Standard bleaching processes are relatively complicated and lengthy as, for example, the bleaching of cotton yarn, which involves substantially seven steps, as follows:—boiling in 10 caustic, as 2% caustic soda, 1% silicate and 1% sulphonated oil or the like, dropping the above bath and washing in hot water, dropping and running through hypochlorite solution,  $\frac{1}{2}$  to 2 TW, dropping and washing in warm water, dropping and souring in a hydrochloric acid or sulphuric acid solution or the like, dropping and washing in warm water, dropping and washing in water to which is added bluing.

An object of this invention is to provide a 20 bleaching process which is much shorter than standard processes, and involves fewer steps.

Another object is to provide a bleaching process employing a compound containing oxygen and chlorine which process will inhibit the characteristic action of the chlorine upon the fibers 25 without interfering with the action of the nascent oxygen.

Still another object is to provide an improved bleaching process which will be efficient, even if the material to be bleached contains insoluble oils.

Another object is to provide a bleaching process which will leave the material, such as rayon, cellulose acetate silk and cotton, free of oil stains, 35 chafe marks and so-called niger beads.

Yet another object is to provide a bleaching process which is considerably less expensive than most standard bleaching processes for like material.

40 Other objects and advantages of the invention will be apparent during the course of the following detailed description thereof.

After the material has undergone any preliminary desirable treatment, such as boiling out in 45 order to remove insoluble oils and the like, the material is treated, preferably, to a bath containing water, sodium stearate and sulphonated oil. For example, in this treatment of 100 pounds of 50 hose having solid white bodies, heels, toes and tops, the preferred formula of this bath is:—

220 gallons water  
 2% sodium stearate  
 2% sulphonated oil

55 said percentages being by weight and the pro-

portion of ingredients may vary between 200 and 250 gallons water and between 2% and 3% sodium stearate and like variations in the sulphonated oil.

This treatment preferably continues for substantially ten minutes, with the bath at a temperature between 100° F. and 110° F. whereupon the bath may or may not be dropped and the material treated to a bath containing sodium hypochlorite and a buffer. The latter may be glues, 10 saponified and/or emulsified fats and oils, sulphonated oils, dextrines, glucose, sugar, fatty alcohols, alkali and alkaline salts.

The sodium hypochlorite and buffer may be mixed together in substantially the following 15 proportions:—

95% by weight sodium hypochlorite  
 5% by weight buffer

However, the percentages of sodium hypochlorite 20 may vary between 95% and 99% while the percentages of buffer may vary between 1% and 5%.

As required, the sodium hypochlorite-buffer mixture may be employed already mixed, since it has been found that this mixture does not lose 25 strength even after being kept for a considerable period.

If the first bath is not dropped, from 8% to 10% by weight of the sodium hypochlorite-buffer mixture is added to it and the material treated 30 therein for from 15 to 20 minutes. At the beginning of this last treatment, i. e., at the time the sodium hypochlorite-buffer mixture is added and the material subjected thereto, the temperature of the bath should be substantially 110° F. It 35 may be less, by allowing the first bath to cool slightly below 100° F. to 110° F., but it should not be over 110° F. at the start of the treatment with the sodium hypochlorite-buffer mixture. Very slowly, the temperature should be brought up to 40 between 140° F. and 180° F. so that, at the close of the fifteen to twenty minute period, the temperature of the bath is between 140° F. and 180° F., whereupon the bath is dropped at once and the material washed, for substantially five minutes, 45 in a bath at a temperature between 100° F. and 110° F. which bath may comprise:—

200 to 250 gallons water  
 1% by weight sodium stearate (high titre)  
 A trace bluing

In the event the sodium hypochlorite-buffer mixture is not added to the first bath, the latter is dropped and the material is treated to a bath containing substantially:—

200 to 250 gallons water  
8% to 20% by weight sodium hypochlorite-buffer mixture

5 The treatment in this last bath should be exactly similar to that just outlined.

After treatment as described, the material may be removed from the sodium hypochlorite-buffer mixture bath and suitably dried.

10 In the bleaching of mercerized cotton and rayon yarns, for example, of substantially 100 pounds weight, the material may be boiled out for substantially five minutes in a bath containing:—

15 200 to 250 gallons water  
2% by weight trisodium phosphate  
4% by weight soda ash  
2% by weight sodium stearate (such as green soap 145)

20 Whereupon, the bath is dropped and the material treated to a bath containing substantially:—

100 to 250 gallons water  
2% by weight trisodium phosphate  
2% by weight sodium stearate (such as green soap 145)  
25 10% by weight sodium hypochlorite-buffer mixture

30 It is preferred that, at the start, this bath be at a temperature of substantially 100° F. and maintained at that temperature for about fifteen minutes, whereupon the bath is brought to a boil and boiling maintained for twenty minutes, after which the bath is dropped and the material rinsed in a bath containing about:—

35 100 to 250 gallons water  
2% sodium stearate  
If and as required bluing

40 For bleaching raw stock cotton, the same is, preferably, treated by boiling for one hour in a 5% caustic soda bath, and is then given a hot rinse (180° F. to boiling) for substantially one-half hour after which it is introduced to a bath which includes:—

45 2% soda ash  
1% sodium stearate  
8% sodium hypochlorite-buffer mixture

50 In this treatment of raw stock cotton, the bath last mentioned is maintained at substantially 110° F. for one hour, whereupon the temperature is raised to the boiling point and boiling maintained for substantially forty-five minutes. Thereupon, this bath is dropped, and the material 55 given a good rinse at 120° F., using 1% sodium stearate and bluing, as desired, in the rinse water. After this last rinse, the material may be extracted.

60 In the bleaching of hose with fast-dyed figures, the preferred improved treatment is substantially as follows for 100 pounds hose. A bath is prepared comprising substantially:—

65 200 to 250 gallons water  
2% to 3% sodium stearate  
2% to 3% sulphonated oil

70 The material is treated in this bath, with the latter at a temperature between 100° F. and 110° F. for a period of substantially ten minutes whereupon there is added between 8% to 10% of the sodium hypochlorite-buffer mixture and treatment continued for from fifteen to twenty minutes, whereupon the temperature is raised to, preferably, 180° F. to 190° F. (altho this temperature may vary between 140° F. and 190° F.). The

higher temperature range is maintained for about twelve minutes after which the bath is dropped and fresh water of between 200 and 250 gallons containing from 1% to 2% sodium stearate (high titre), with bluing if desired, is employed as a 5 rinse, the rinse being maintained at a temperature of from 100° F. to 110° F. over a period of substantially five minutes, whereupon the surplus may be extracted and the material dried.

10 In the treatment of material with acetate figures, such as hose, 100 pounds of such material may be treated to:—

200 to 250 gallons water  
2% to 3% sodium stearate  
2% to 3% sulphonated oil

15

This treatment may continue for substantially ten minutes at from 100° F. to 110° F. after which acetate dyes may be added and treatment continued for substantially thirty minutes at a temperature varying between 160° F. and 170° F. At the expiration of this period the bath is dropped and fresh water added at a temperature of between 100° F. and 110° F., the water containing substantially 1% sodium stearate and 8% to 25 10% sodium hypochlorite-buffer mixture. The material is maintained in this bleaching bath for substantially fifteen minutes with the temperature of the bath at between 100° F. and 110° F., whereupon the temperature is increased, over a 30 period of substantially fifteen minutes to about 170° F. after which this treatment is discontinued, the bath dropped, and fresh water at about 110° F. employed as a rinse, this water containing about 1% sodium stearate to 200 to 250 gallons 35 of water. A period of between five and ten minutes will be sufficient to remove all surplus dyes.

With the treatment described, the chlorine does not attack the material being bleached, due to the proportions of buffers employed and the temperatures maintained.

40 Various changes may be made to the forms of the invention herein described, without departing from the spirit of the invention or the scope of the claims.

45 What is claimed is:

1. In a bleaching process for fibrous cellulose containing material, the steps which consist in subjecting said material over a period of between ten and twenty minutes to a bath containing 50 sodium hypochlorite and a buffer, said bath being at a temperature between 100° F. and 110° F., and subsequently bringing the temperature of said bath up to between 140° F. and the boiling temperature of said bath over a period of between 55 twelve minutes and forty-five minutes, and dropping said bath, said bath being the sole major bleaching step of said process.

2. In a bleaching process for rayon, cotton, cellulose acetate silks and like material, the steps 60 of freeing said material of stains, chafe marks and so-called niger beads thereon, which consist in subjecting said material over a period of between ten and twenty minutes to a bath consisting of sodium hypochlorite, a buffer and water, 65 said bath being at a temperature of between 100° F. and 110° F., and subsequently gradually increasing this temperature over a period of between fifteen and twenty minutes until the temperature reaches between 160° F. and 180° F. and 70 immediately separating said material and said bath.

3. A bleaching process for rayon, cotton, cellulose acetate silks and like material, which consists in subjecting said material over a period of 75

between ten and twenty minutes to a bath consisting of water, sodium stearate and sulphonated oil at a temperature of between 100° F. and 110° F., dropping said bath, and subsequently subjecting said material to a bath containing sodium hypochlorite and a buffer at a temperature of substantially 110° F., bringing said second bath, over a period of between fifteen and twenty minutes, to a temperature of between 160° F. and 180° F., dropping said bath, and washing said material.

4. A bleaching process for fibrous cellulose material containing acetate figures, which consists in treating said material to a bath comprising

water, sodium stearate and sulphonated oil for substantially ten minutes at a temperature between 100° F. and 110° F., adding acetate dyes, increasing said temperature to between 160° F. and 170° F., maintaining said temperature for substantially thirty minutes, dropping said bath, and treating said material to a bath comprising water, sodium stearate, sodium hypochlorite and a buffer at a temperature between 100° F. and 110° F. for substantially fifteen minutes, slowly increasing said temperature, over a period of substantially fifteen minutes, to substantially 170° F., and immediately dropping said bath.

EDWIN P. SHERMAN.